

S. T. WELLMAN.  
MANUFACTURE OF INGOTS.  
APPLICATION FILED MAR. 27, 1913.

1,081,997.

Patented Dec. 23, 1913.



# UNITED STATES PATENT OFFICE.

SAMUEL T. WELLMAN, OF CLEVELAND, OHIO, ASSIGNOR TO THE LIQUID FORGED STEEL COMPANY, OF CLEVELAND, OHIO.

## MANUFACTURE OF INGOTS.

1,081,997.

Specification of Letters Patent. Patented Dec. 23, 1913.

Application filed March 27, 1913. Serial No. 757,052.

To all whom it may concern:

Be it known that I, SAMUEL T. WELLMAN, a citizen of the United States, residing at Cleveland, in the county of Cuyahoga and 5 State of Ohio, have invented a certain new and useful Improvement in Manufacture of Ingots, of which the following is a full, clear, and exact description.

The object of this invention is to cast 10 sound ingots, that is to say, ingots which are substantially free from segregation and piping.

It is in the nature of an improvement 15 upon that process of producing ingots which includes the pouring of the metal into a tapered mold, whose large end is uppermost, and in jarring said metal, while it is solidifying, by a succession of vertical impacts.

Practical difficulties have been encountered in making sound ingots in the manner 20 stated. The metal in contact with the walls of the mold first solidifies, thereby forming a shell, which at first fits snugly against the tapered walls of the mold. But as the solidification proceeds, this shell cools, and shrinks 25 away from the said walls. This takes place before the middle part of the mold has become solid, and while the jarring of the metal is being continued. In fact, it is the 30 jarring during the final solidification of the metal which is most efficient in preventing piping. After the metal shell has shrunk away from the side walls of the mold and the jarring is continued, the still molten or 35 pasty metal in the shell will be caused to settle down in the shell; and so much lateral pressure will be produced thereby, that in many cases, the ingot shell will be split lengthwise. The splitting likewise pulls 40 apart the pasty center of the shell and produces therein holes, which while not like the ordinary pipes, are nevertheless quite as 45 objectionable.

The object of this invention is to prevent 45 the splitting of ingots, while they are solidifying in a tapered mold, whose smaller end is down, and while the ingot is being subjected to the jarring action of repeated vertical impacts.

In the drawings, Figure 1 is a central longitudinal section of a mold and associated apparatus, in which the invention 50 is embodied, and by which it may be practised. Fig. 2 is a transverse sectional view in the plane indicated by line 2—2 on Fig.

1. Fig. 3 is a transverse sectional view in the plane indicated by line 3—3 on Fig. 1.

In carrying out the invention, a tapered mold A is employed, said mold being largest at its upper end. The lower portion of the 60 mold cavity, from the point marked *a* downward, may, and, preferably, does have vertical side walls. There is preferably also a hole *a*<sup>1</sup> in the bottom of the mold. This hole is covered by a bottom plate B having a projection *b* which fits in the hole *a*<sup>1</sup>. While as stated the best construction involves the use of a mold whose cavity at its lower end has vertical instead of tapered walls, and while it is advantageous to have the movable 70 bottom plate B, and to employ also a downwardly movable plate C which fits in the lower part of the mold cavity, these are minor features of the invention. The primary features of the invention are that the 75 mold is partially filled by dry, free flowing sand D, which rests upon the plate B, and in turn supports the plate C; and that in the lower end of the mold there is an opening *a*<sup>2</sup> or a plurality of such openings through 80 which this sand may slowly flow out.

E represents a conical pointed valve which screws through a lug *f* fixed to the side of a sand delivery spout F, so that by turning this valve, the area of the discharge opening for 85 the sand may be varied as required to enable the same to flow out at the desired rate. The construction described is associated with each of the openings *a*<sup>2</sup>.

The mold has at its lower end ears *a*<sup>3</sup>, by 90 which the mold is secured to the vertically vibrating horizontal table *g*. This table is formed on the upper end of a vertically reciprocating piston G, which is movable vertically in a fixed cylinder H mounted on a 95 suitable foundation J. K represents a valve casing which contains a valve to control the inflow and outflow of compressed air through the port *h*. This pneumatic cylinder and piston as a means for moving the 100 mold up, and allowing it to fall so that when the lower end of the piston strikes the bottom of the cylinder, the mold and metal therein will be jarred as by vertical impact, is of familiar construction, and not a part 105 of the present invention.

When a sufficient quantity of sand has been put into the mold, and the plate C has also been put into the mold resting upon this sand, the molten metal is poured in. 110

While it is solidifying, the jarring mechanism is in operation. When the shell of metal has formed in the mold in contact with the walls, and is thickening, through 5 the solidifying of the metal near the center, the shell will begin to shrink. The valves E should be so adjusted that the sand will flow out fast enough to allow this shrinking ingot to settle down in the mold, and to there- 10 by always maintain contact with the walls thereof. As the shrinking ingot settles down in the tapered mold it will for a time be compressed laterally to a small degree, but enough to force the still fluid or pasty 15 metal upward so as to fill what might otherwise become a permanent pipe. It has been found of advantage in producing this compression to put a heavy weight W in the top of the mold resting upon the metal 20 therein.

The purpose of the plate C is to keep the metal from direct contact with the sand. And the purpose of the bottom plate B and its downward projection through hole 25  $a^1$  is to afford a convenient means by which the solidified ingot may be forced upwardly in the mold for the purpose of removal.

Having described my invention, I claim:

1. The process of forming sound ingots 30 which consists in pouring the molten metal into a tapered mold whose large end is uppermost and which has in its bottom a quantity of free flowing sand, in jarring the mold while the molten metal is solidifying, 35 and in allowing the sand to flow out through a hole in the mold wall at a rate such as will

allow the shrinking ingot shell to settle down in the mold and maintain contact with the side walls thereof.

2. In ingot forming mechanism, the combination of a tapered mold whose large end is uppermost, and which has a hole through its wall near its lower end, a mass of free flowing sand in the bottom of said mold, and means for jarring the mold while it 45 contains solidifying molten metal.

3. In ingot forming mechanism, the combination of a tapered mold whose large end is uppermost, and which has a hole through its wall near its lower end, a mass of free 50 flowing sand in the bottom of said mold, means for jarring the mold while it contains solidifying molten metal, and a valve to control the rate at which the same is allowed to flow out through said hole.

4. In ingot forming mechanism, the combination of a mold whose mold cavity has vertical walls at the lower end thereof, and above them walls which regularly diverge toward the top,—said mold having a hole through its wall near the bottom of said mold cavity, a mass of free flowing sand in the bottom of said mold cavity, a plate which rests upon said sand and forms the bottom of the metal receiving part of the mold cavity, and means for jarring the mold.

In testimony whereof, I hereunto affix my signature in the presence of two witnesses.

SAMUEL T. WELLMAN.

Witnesses:

E. B. GILCHRIST,  
E. L. THURSTON.